# EUROPEAN PATENT SPECIFICATION

(11) **EP 0 099 617 B1**
(45) Date of publication and mention of the grant of the patent: **30.12.1986**
(21) Application number: 83302009.2
(22) Date of filing: 11.04.1983
(51) Int. Cl.: C21D 8/12, H01F 1/16

(54) **Method for producing cube-on-edge oriented silicon steel**
Verfahren zur Herstellung von kornorientiertem Siliciumstahl mit Goss-Textur
Procédé de fabrication d'acier au silicium à grains orientés cube-sur-arête

(30) Priority: 19.07.1982 US 399674
(43) Date of publication of application: 01.02.1984
(73) Proprietor: ALLEGHENY LUDLUM STEEL CORPORATION, Pittsburgh Pennsylvania 15222 (US)
(72) Inventor: Miller, Robert Frederick, Evans City Pennsylvania 16033 (US)
(74) Representative: Sheader, Brian N.

## Description

This invention relates to a method of producing cube-on-edge oriented silicon steel.

Cube-on-edge oriented silicon steel, in the form of sheets, is known for use in various electrical applications, including the manufacture of transformer cores. With cube-on-edge silicon steel the alloy is characterized by secondary recrystallization in the (110) (001) position, which is termed the cube-on-edge position. This material in sheet form has the direction of easy magnetization in the direction of rolling. In applications for this material, and specifically when used in the manufacture of transformer cores, the material is required to have reduced watt loss, because the consumption of electrical energy decreases as iron loss decreases. Reduced watt loss may be promoted by achieving fine secondary grain size during texture annealing. One such method of producing cube-on-edge oriented silicon steel in sheet form is disclosed in British Patent No. GB-A-610 440.

It is accordingly an object of the present invention to provide a method whereby cube-on-edge silicon steel may be provided with a fine secondary grain or crystal structure after texture annealing, which achieves reduced watt loss.

The present invention provides a method of producing cube-on-edge oriented silicon steel having reduced watt loss, including the steps of hot-rolling, cold-rolling with intermediate annealing to final gauge, decarburizing, and final texture annealing, characterised by providing a cold-rolling deformation to the steel to achieve a 0.5% to 15% elongation of the decarburized steel prior to said final texture annealing.

With respect to cube-on-edge silicon steel to which the present invention is directed, this steel is conventionally processed by hot rolling followed by one or more cold rolling operations with intermediate anneals. After cold rolling the steel is subjected to a normalizing operation to achieve primary recrystallization and decarburization. Typically, normalizing is conducted at temperatures with the range of 704 to 871°C (1300 to 1600°F). In accordance with the invention, after normalizing the steel is subjected to cold deformation as by a cold-rolling operation. After cold deformation, the steel is final texture annealed in the conventional manner to achieve secondary recrystallization. It has been found that by cold deforming in accordance with the invention following normalizing and prior to texture annealing secondary grain growth is inhibited during final texture annealing, which results in reduced watt loss. For this purpose, cold rolling to achieve an elongation within the range of 0.5 to 15% has been found to be effective for the purpose. It has been found that by varying the amount of cold reduction the grain size after texture annealing may be regulated. Although the practice of the invention finds utility with cube-on-edge silicon steels generally it is particularly adapted to steels of this type within the following composition limits in percent by weight:

By way of specific example two heats of the alloy identified SX-14 (Heat Nos. 154684 and 153595) were melted to the following composition in percent by weight:

This material was processed in the conventional manner by hot rolling followed by a cold-rolling operation. Then it was subjected to a final normalizing treatment comprising continuous annealing at a temperature of 800°C (1475°F) which served to decarburize the steel and effect primary recrystallization. The normalized steel in strip form was cut to lengths suitable for cold rolling and rolled in a 4-high cold rolling mill at ambient temperature. The extent of plastic deformation was determined by measuring the percent elongation over a 610 mm (24") span scribed on the steel strip before cold rolling. For control purposes samples of the steel were retained prior to cold rolling, and elongation F for Heat No. 153595 is included in Table 1 for comparison purposes. The material was cut into standard Epstein strip samples and roller coated with a water slurry of MgO+ .75%B. Texture annealing was performed in dry hydrogen. The anneal cycle consisted of charging the steel into a furnace at 1400°F (760°C), heating at 50°F (28°C) per hour to 2150°F (1175°C), holding 20 hours at 2150°F (1175°C) and furnace cooling. Magnetic testing and grain size measurements were made after this texture annealing operation. Table I lists the magnetic properties and grain size of the material tested.

The method of the present invention reduces both the permeability at high induction levels and the size of the grains formed during final texture annealing. The current trend in electrical steel usage is toward lower inductions and significant improvements have been made in lowering core losses or watt losses by reducing the sheet thickness. Commercially available material typically ranges from .014 to .011 inch (.35 to .28 mm), and may be .009 inch (.23 mm) and lower.

As such materials are used at lower inductions, of the order of 15 kilogauss or lower, the reduction in permeability at high inductions becomes less important in electrical equipment. Also, as the sheet thicknesses are reduced, core losses arising from eddy currents appear to be more dependent upon the material grain size, i.e., core losses decrease with decreasing grain size. The advantages of the present invention establish that it is of substantial importance in the manufacture of thin sheet, of the order of less than .015 inch to .004 inch (.38 to .1 mm) thick, and suitable for use in transformers.

## Claims

1. A method of producing cube-on-edge oriented silicon steel characterised by reduced watt loss, including the steps of hot-rolling, cold-rolling with intermediate annealing to final gauge, decarburizing, and final texture annealing, characterized in providing a cold-rolling deformation to the steel to achieve a 0.5% to 15% elongation of the decarburized steel prior to said final texture annealing.

2. A method according to claim 1, characterised in that the steel is normalized at a temperature within the range of 704 to 871°C (1300 to 1600°F).

3. A method according to claim 1 or 2, characterised in that the steel falls within the following composition limits in percentage by weight.

4. A method according to claim 1 or 2, characterised in that the steel falls within the following composition limits in percentage by weight:

5. A method according to any one of the preceding claims, characterised in that the steel has a thickness of less than 0.38 mm (0.015 inch).

## Patentansprüche

1. Verfahren zum Herstellen eines durch verminderten Kernverlust charakterisierten Siliciumstahls mit Goss-Textur, umfassend die Schritte des Warmwalzens, Kaltwalzens mit Zwischenglühung auf Endabmessung, Entkohlens und Schlußtexturglühens, dadurch gekennzeichnet, daß der Stahl so kaltgewalzt wird, daß eine 0,5 bis 15 %ige Dehnung des entkohlten Stahls vor der Schlußtexturglühung erreicht wird.

2. Verfahren nach Anspruch 1, dadurch gekennzeichnet, daß der Stahl bei einer Temperatur innerhalb des Bereiches von 704 bis 871°C (1 300 bis 1 600°F) normalisiert wird.

3. Verfahren nach Anspruch 1 oder 2, dadurch gekennzeichnet, daß der Stahl in die folgenden Zusammensetzungsbereiche (Gew.-%) hineinfällt:

4. Verfahren nach Anspruch 1 oder 2, dadurch gekennzeichnet, daß der Stahl in die folgenden Zusammensetzungsbereiche (Gew.-%) hineinfällt:

5. Verfahren nach einem der vorhergehenden Ansprüche, dadurch gekennzeichnet, daß der Stahl eine Dicke von weniger als 0,38 mm (0,015 Zoll) aufweist.

## Revendications

1. Procédé pour la fabrication d'acier au silicium à orientation de Goss, caractérisé par une réduction des pertes d'énergie active, comprenant les étapes de laminage à chaud, laminage à froid avec recuit intermédiaire à l'épaisseur calibrée finale, décarburation et recuit de texture final, caractérisé en ce que l'on donne à l'acier une déformation par laminage à froid pour obtenir un allongement de 0,5 à 15% de l'acier décarburé avant ledit recuit de texture final.

2. Procédé selon la revendication 1, caractérisé en ce que l'acier est normalisé à une température comprise dans la gamme de 704 et 871°C (1 300 à 1 600°F).

3. Procédé selon la revendication 1 ou 2, caractérisé en ce que l'acier est compris dans les limites de composition suivantes, en pour-cent en poids:

4. Procédé selon la revendication 1 ou 2, caractérisé en ce que l'acier est compris dans les limites de composition finales en pour-cent en poids:

5. Procédé selon l'une quelconque des revendications précédentes, caractérisé en ce que l'acier a une épaisseur moins de 0,38 mm (0,015 pouce).
